

# United States Patent [19]

Wendler et al.

[11] 3,849,322

[45] Nov. 19, 1974

[54] ALKYLATED TERTIARY AMINES AS HIGH-TEMPERATURE ANTIOXIDANTS FOR ESTER BASE LUBRICANTS

[75] Inventors: Kenneth T. Wendler, Freehold; David A. Daniels, Kendall Park, both of N.J.

[73] Assignee: W. R. Grace & Co., New York, N.Y.

[22] Filed: July 16, 1973

[21] Appl. No.: 379,823

## Related U.S. Application Data

[63] Continuation-in-part of Ser. No. 362,693, May 22, 1973, abandoned, which is a continuation of Ser. No. 152,405, June 11, 1971, abandoned.

[52] U.S. Cl..... 252/49.9, 252/51.5 R, 252/51.5 A, 252/50, 252/401, 260/570.8 R, 260/570.9

[51] Int. Cl..... C10m 1/34

[58] Field of Search..... 252/50, 51, 51.5 R, 51.5 A, 252/46.7, 49.9, 401, 403, 565; 260/570.9

## [56] References Cited

### UNITED STATES PATENTS

2,722,518 11/1955 Watson ..... 252/46.7

|           |         |                     |          |
|-----------|---------|---------------------|----------|
| 2,758,086 | 8/1956  | Stuart et al. ....  | 252/32.5 |
| 2,930,758 | 3/1960  | Tierney et al. .... | 252/46.7 |
| 3,231,499 | 1/1966  | Smith.....          | 252/565  |
| 3,305,483 | 2/1967  | Coffield .....      | 252/42.4 |
| 3,413,227 | 11/1968 | Howard et al. ....  | 252/51.5 |
| 3,663,436 | 5/1972  | Carswell .....      | 252/28   |

## FOREIGN PATENTS OR APPLICATIONS

793,115 4/1958 Great Britain .....

Primary Examiner—W. Cannon  
Attorney, Agent, or Firm—Elton Fisher; Kenneth E. Prince

## [57] ABSTRACT

This invention is directed to an improved ester base lubricant composition which exhibits enhanced oxidative stability in use. This improved lubricant composition comprises a major amount of an ester of a carboxylic acid and a minor amount of; (a) a mixture of a secondary aromatic amine and a tertiary aromatic amine; or (b) a mixture of two tertiary aromatic amines. Other additives can be included in the improved lubricant composition.

40 Claims, No Drawings

ALKYLATED TERTIARY AMINES AS  
HIGH-TEMPERATURE ANTIODANTS FOR  
ESTER BASE LUBRICANTS

CROSS REFERENCE TO RELATED APPLICATION

This is a continuation-in-part of our copending application Ser. No. 362,693, filed May 22, 1973 and now abandoned which is a continuation of application Ser. No. 152,405, filed June 11, 1971 and now abandoned.

BACKGROUND OF THE INVENTION

The instant invention is directed to an improved lubricant composition based on a lubricant ester (e.g., a lubricant comprising a lubricant ester of a carboxylic acid--especially an ester of an alkanedioic acid). Said improved lubricant composition comprises a major amount of such ester plus a minor amount of; (a) a secondary amine selected as recited infra plus a tertiary amine selected as recited infra; or (b) two tertiary amines selected as recited infra. Said improved lubricant composition exhibits superior oxidative stability at elevated temperatures.

Petroleum oil lubricants have been known to the art for some time and have proven useful for general purpose lubrication. However, petroleum oils have generally been unsatisfactory lubricants in service at temperatures much above 200°F to 250°F because of a tendency of such lubricants to oxidize rapidly. A variety of synthetic lubricants have been developed in the past several decades to deal with high temperature and related lubricant use requirements. The ever increasing development of higher speed and heavier duty military and industrial equipment has produced an ever increasing demand to develop improved lubricants.

Since about 1940, ester base lubricants have been available to the art and have been used with some success for high temperature lubrication. With the development of jet engines and particularly high-temperature jet engines, increasing use has been made of synthetic lubricants based on organic esters of the diester type such as those diesters derived from adipic, azelaic and sebacic acids by esterification with C<sub>8</sub> to C<sub>10</sub> alkanols. An example of a diester fluid which has been a widely used synthetic lubricant is di(2-ethylhexyl) sebacate which has been employed in lubricant formulations known in the art as jet engine oils and related lubricants. However, recent heavy demands and price competition have led to use of a variety of diesters derived from more readily available di-carboxylic acids.

Synthetic ester based lubricant compositions (e.g., an ester base lubricant plus an additive or additives) which include phosphate esters are known to those skilled in the art. These organic phosphorus compounds have the general formula OP(OR)<sub>3</sub> where R represents an aryl or an alkyl group or the like. Improved load carrying capacity and wear protection for gears and ball and roller bearings has been provided by including from about 1 to about 5 weight percent tricresyl phosphate in the lubricant composition of our invention.

Various known synthetic lubricating compositions have often included secondary amines with some success for stabilization against oxidation. Typically, phenothiazine has been included in an amount of about 0.5 weight percent. These compositions have generally included substantial quantities of various expensive ma-

terials for use as thickening agents, rust inhibitors and as other special purpose agents. However, many of these known ester based lubricant compositions have not been entirely satisfactory in high temperature service due to rapid oxidation of the lubricant resulting in excessive increase in viscosity with increasing temperature, excessive deposit formation resulting from degradation of the lubricant, high corrosion-induced weight losses for the materials being lubricated and for other reasons. Moreover, many of these otherwise suitable lubricating compositions have not met the recently more stringent oxidative stability and related recently more critical requirements of lubricant users.

U.S. Pat. No. 3,282,840 (Foster, et al, 252/50) teaches a lubricating composition which is a carboxylic acid ester lubricant stabilized with a secondary amine such as diphenylamine, p,p'-dioctylidiphenylamine, phenyl- $\alpha$ -naphthylamine, and the like.

U.S. Pat. No. 3,305,483 (Coffield, 252/42.4) teaches the use of certain tertiary amines to stabilize lubricating oil, gear oil, grease, and rubber.

U.S. Pat. No. 3,660,290 (Schloobohm, 252/51.5A) teaches the use of certain 4-alkylphenyl-1-alkyl-2-naphthylamines and mixtures thereof with certain 4-alkyl-phenyl-2-naphthylamines to improve the oxidation resistance of certain lubricant compositions. Certain other additives including phosphorus extreme pressure agents and a triazole corrosion inhibitor are included in some of the lubricant compositions taught by said patent.

Other patents teaching lubricant compositions based on esters of carboxylic acids include:

1. U.S. Pat. No. 2,758,086 (Stewart, et al., 252/32.5).
2. U.S. Pat. No. 3,663,436 (Carswell, 252/28).
3. U.S. Pat. No. 3,413,227 (Howard, et al., 252/51.4).
4. U.S. Pat. No. 2,722,518 (Watson, 252/46.7).
5. U.S. Pat. No. 1,930,758 (Tierney, et al., 252/46.7).
6. British Pat. No. 793,115 (Esso Research and Engineering Company).

Ester lubricants (lubricant esters of carboxylic acids) are also taught by the Kirk-Othmer Encyclopedia of Chemical Technology. See Volume 8; page 514 of the first edition and Volume 12, pages 579-580 and Table 10 (on page 578) of the second edition of said Encyclopedia.

SUMMARY OF THE INVENTION

In summary, this invention is directed to an improvement in a lubricant composition comprising an ester type lubricant (an ester base lubricant, e.g., a lubricant composition comprising a lubricant ester of a carboxylic acid), said improvement comprising the presence of;

- a. a secondary amine having the formula;



in which  $R_1$  and  $R_2$  are separately alkyl groups having 4-12 carbon atoms; and  
b. a tertiary amine having the formula;



or



in which  $R_4$  is an alkyl group having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen,  $A$  is  $CCl_2$ ,  $CBr_2$ ,  $Cl_2$ , or an alkylene group having about 1-7 carbon atoms, and  $R_9$  is hydrogen or an alkyl group having 4-12 carbon atoms, said secondary amine and said tertiary amine being present in an amount effective for improving oxidative stability of the ester base lubricant at temperatures up to at least 400°F.

The amount of said amines present in the ester base lubricant is not critical and a finite amount produces a finite improvement; however, we generally prefer to have about 0.5-8 (preferably 0.5-7) parts of said secondary amine and 0.5-10 (preferably 0.5-8) parts of said tertiary amine present per 100 parts of said ester.

#### DESCRIPTION OF PREFERRED EMBODIMENTS

In a preferred embodiment ("Embodiment A") this invention is directed to an improvement in a lubricant composition comprising an ester type lubricant (an ester base lubricant, e.g., a lubricant composition comprising a lubricant ester of a carboxylic acid), said improvement comprising the presence of;

(a) a first tertiary amine having the formula



in which  $R_4$  and  $R_5$  are separately alkyl groups having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen, and  $A$  is  $CCl_2$ ,  $CBr_2$ ,  $Cl_2$ , or an alkylene group having about 1-7 carbon atoms, and

15 b. a second tertiary amine selected from the group consisting of tertiary amines having the formula



in which  $R_4$  is an alkyl group having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen, and  $A$  is  $CCl_2$ ,  $CBr_2$ ,  $Cl_2$ , or an alkylene group having about 1-7 carbon atoms, and  $R_9$  is hydrogen or an alkyl group having 4-12 carbon atoms, said first tertiary amine and said second tertiary amine being present in an amount effective for improving oxidative stability of the ester base lubricant at temperatures up to at least 400°F. The amount of said amines present in the ester base lubricant is not critical and a finite amount produces a finite improvement; however, we generally prefer to have about 0.5-10 parts of said second tertiary amine present per 100 parts of said ester (the lubricant ester of the carboxylic acid), and we generally prefer a weight ratio of first tertiary amine to second tertiary amine of about

55 1:2-4.

60 In another preferred embodiment ("Embodiment a-1") this invention is directed to an improvement in a lubricant composition comprising an ester type lubri-

65

cant (an ester base lubricant, e.g., a lubricant composition comprising a lubricant ester of carboxylic acid), said improvement comprising the presence of;

a. a secondary amine having the formula;



in which  $R_1$  is an alkyl group having 4-12 carbon atoms and  $R_3$  is hydrogen or an alkyl group having 4-12 carbon atoms; and

b. a tertiary amine having the formula;



in which  $R_4$  and  $R_5$  are separately alkyl groups having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen,  $A$  is  $CCl_2$ ,  $CBr_2$ ,  $Cl_2$ , or an alkylene group having about 1-7 carbon atoms, said secondary amine and said tertiary amine being present in an amount effective for improving oxidative stability of the ester base lubricant at temperatures up to at least 400°F.

In preferred embodiments of; (a) the embodiment (lubricant composition) set forth in the above Summary; and (b) the embodiments (i.e., the lubricant composition) set forth in Embodiments A and A-1, supra:

1.  $R_1$ ,  $R_2$ , and  $R_3$  are alkyl groups having 8 carbon atoms and are more preferably alkyl groups having the formula  $C(CH_3)_2CH_2C(CH_3)_3$  or  $CH_2C(CH_3)_2C(CH_3)_3$ .

2.  $R_4$ ,  $R_5$ , and  $R_9$  are alkyl groups having 8 carbon atoms and are more preferably alkyl groups having the formula  $C(CH_3)_2CH_2C(CH_3)_3$  or  $CH_2C(CH_3)_2C(CH_3)_3$ .

3. The lubricant composition contains 0-10 (preferably 0.5-10) parts of a phosphorus-containing ester per 100 parts of the lubricant ester of a carboxylic acid. Preferred phosphorus-containing esters are tri-esterified phosphoric acid components derived from a hydroxy compound selected from the group consisting of straight and branched chain alcohols having from 1 to about 8 carbon atoms, phenol, cresols, xylenols, and alkyl substituted naphthols in which the alkyl groups each have 1-10 carbon atoms in straight or branched chain configuration, and the number of alkyl groups is 1-3. Especially preferred phosphorus-containing acid esters include tricresyl phosphate, triphenyl phosphate, cresyldiphenyl phosphate, xylodiphenyl phosphate, triethyl phosphate, tributyl phosphate, and triisooctyl phosphate. 4. The lubricant composition includes, or contains, 0 to 1 part, per 100 parts of the lubricant, of an amino substituted 1,2,4-triazole component, benzotriazole, 5,5-methylene-bis-(1,2,3-benzotriazole), or an alkyl benzotriazole in which the alkyl group contains about 1-12 carbon atoms.

5. The carboxylic acid ester component of the lubricant composition is acid ester component is a diester having the general formula  $R_{11}OOC(CH_2)_nCOOR_{10}$  wherein  $n$  is an integer from 2-30 and  $R_{11}$  and  $R_{10}$  are separately selected from the group consisting of straight and branched chain alkyl groups containing from 6-16 carbon atoms. It is especially preferred that  $R_{11}$  and  $R_{10}$  are separately selected from the group consisting of straight and branched chain octyl and tridecyl groups and  $n$  is 4-8.  $R_{10}$  and  $R_{11}$  can be identical.

6. The carboxylic acid ester component of the lubricant composition is an ester derived from aliphatic carboxylic acids having 3-18 carbon atoms and polyols selecting from the group consisting of trimethylolpropane, pentaerythritol, dipentaerythritol, tripentaerythritol and neopentylglycol.

In especially preferred embodiments of our invention as recited in the above Summary:

40 1. The secondary amine can be selected from: 4,4'-(1,1,3,3-tetramethylbutyl)-diphenylamine, N-4-(1,1,3,3-tetramethylbutyl)-phenyl- $\alpha$ -naphthylamine, N-4-(1,1,3,3-tetramethylbutyl)-phenyl- $\beta$ -naphthylamine, and N-4-(1,1,3,3-tetramethylbutyl)-phenyl-1-(1,1,3,3-tetramethylbutyl)- $\beta$ -naphthylamine.

45 2. The tertiary amine can be selected from: N,N-bis-4-(1,1,3,3-tetramethylbutyl)-phenylbenzylamine, N,N-bis-4-(1,1,3,3-tetramethylbutyl)-phenyl-2-phenylethylamine, N,N-bis-4-(1,1,3,3-tetramethylbutyl)-phenyl-4-methylbenzylamine, N,N-bis-4-(1,1,3,3-tetramethylbutyl)-phenyl-2-chlorobenzylamine, N,N-bis-4-(1,1,3,3-tetramethylbutyl)-phenyl-4-chlorobenzylamine, N,N-bis-4-(1,1,3,3-tetramethylbutyl)-phenyl-2,4-dichlorobenzylamine, N,N-bis-4-(1,1,3,3-tetramethylbutyl)-phenyl-3,4-dichlorobenzylamine, N,N-bis-4-(1,1,3,3-tetramethylbutyl)-phenyl- $\alpha$ -dichlorobenzylamine, N,N-bis-4-(1,1,3,3-tetramethylbutyl)-phenyl-2-fluorobenzylamine, N,N-bis-4-(1,1,3,3-tetramethylbutyl)-phenyl-4-fluorobenzylamine, N,N-bis-4-(1,1,3,3-tetramethylbutyl)-phenyl-4-nitrobenzylamine, N,N-bis-4-(1,1,3,3-tetramethylbutyl)-phenyl-2,2-dimethyl-2-phenylethylamine, N-4-(1,1,3,3-tetramethylbutyl)-phenyl-N- $\alpha$ -naphthylbenzylamine, N-4-(1,1,3,3-

50 55 60 65

tetramethylbutyl)-phenyl-N- $\alpha$ -naphthyl-2-phenylethylamine, N-4-(1,1,3,3-tetramethylbutyl)-phenyl-N- $\alpha$ -naphthyl-2-methylbenzylamine, N-4-(1,1,3,3-tetramethylbutyl)-phenyl-N- $\alpha$ -naphthyl-4-methylbenzylamine, N-4-(1,1,3,3-tetramethylbutyl)-phenyl-N- $\alpha$ -naphthyl-2-chlorobenzylamine, N-4-(1,1,3,3-tetramethylbutyl)-phenyl-N- $\alpha$ -naphthyl-4-chlorobenzylamine, N-4-(1,1,3,3-tetramethylbutyl)-phenyl-N- $\alpha$ -naphthyl-2,4-dichlorobenzylamine, N-4-(1,1,3,3-tetramethylbutyl)-phenyl-N- $\alpha$ -naphthyl-3,4-dichlorobenzylamine, N-4-(1,1,3,3-tetramethylbutyl)-phenyl-N- $\alpha$ -naphthyl- $\alpha$ ,  $\alpha$ -dichlorobenzylamine, N-4-(1,1,3,3-tetramethylbutyl)-phenyl-N- $\alpha$ -naphthyl-2-fluorobenzylamine, N-4-(1,1,3,3-tetramethylbutyl)-phenyl-N- $\alpha$ -naphthyl-4-fluorobenzylamine, N-4-(1,1,3,3-tetramethylbutyl)-phenyl-N- $\alpha$ -naphthyl-4-nitrobenzylamine, N-4-(1,1,3,3-tetramethylbutyl)-phenyl-N- $\beta$ -naphthylbenzylamine, N-4-(1,1,3,3-tetramethylbutyl)-phenyl-N- $\beta$ -naphthyl-2-phenylethylamine, N-4-(1,1,3,3-tetramethylbutyl)-phenyl-N- $\beta$ -naphthyl-2-methylbenzylamine, N-4-(1,1,3,3-tetramethylbutyl)-phenyl-N- $\beta$ -naphthyl-4-methylbenzylamine, N-4-(1,1,3,3-tetramethylbutyl)-phenyl-N- $\beta$ -naphthyl-2-chlorobenzylamine, N-4-(1,1,3,3-tetramethylbutyl)-phenyl-N- $\beta$ -naphthyl-4-chlorobenzylamine, N-4-(1,1,3,3-tetramethylbutyl)-phenyl-N- $\beta$ -naphthyl-2,4-dichlorobenzylamine, N-4-(1,1,3,3-tetramethylbutyl)-phenyl-N- $\beta$ -naphthyl-3,4-dichlorobenzylamine, N-4-(1,1,3,3-tetramethylbutyl)-phenyl-N- $\beta$ -naphthyl- $\alpha$ ,  $\alpha$ -dichlorobenzylamine, N-4-(1,1,3,3-tetramethylbutyl)-phenyl-N- $\beta$ -naphthyl-2-fluorobenzylamine, N-4-(1,1,3,3-tetramethylbutyl)-phenyl-N- $\beta$ -naphthyl-4-fluorobenzylamine, N-4-(1,1,3,3-tetramethylbutyl)-phenyl-N- $\beta$ -naphthyl-4-nitrobenzylamine, N-4-(1,1,3,3-tetramethylbutyl)-phenyl-N-1-(1,1,3,3-tetramethylbutyl)- $\beta$ -naphthylbenzylamine, N-4-(1,1,3,3-tetramethylbutyl)-phenyl-N- $\beta$ -naphthyl-2,2-dimethyl-2-phenylethylamine.

In our invention as recited in Embodiment A, supra:

1. The first tertiary amine can be selected from: N,N-bis-4-(1,1,3,3-tetramethylbutyl)-phenylbenzylamine N,N-bis-4-(1,1,3,3-tetramethylbutyl)-phenyl-2-phenylethylamine, N,N-bis-4-(1,1,3,3-tetramethylbutyl)-phenyl-2-methylbenzylamine, N,N-bis-4-(1,1,3,3-tetramethylbutyl)-phenyl-4-methylbenzylamine, N,N-bis-4-(1,1,3,3-tetramethylbutyl)-phenyl-2-chlorobenzylamine, N,N-bis-4-(1,1,3,3-tetramethylbutyl)-phenyl-4-chlorobenzylamine, N,N-bis-4-(1,1,3,3-tetramethylbutyl)-phenyl-2,4-dichlorobenzylamine, N,N-bis-4-(1,1,3,3-tetramethylbutyl)-phenyl-3,4-dichlorobenzylamine, N,N-bis-4-(1,1,3,3-tetramethylbutyl)-phenyl- $\alpha$ ,  $\alpha$ -dichlorobenzylamine, N,N-bis-4-(1,1,3,3-tetramethylbutyl)-phenyl-2-fluorobenzylamine, N,N-bis-4-(1,1,3,3-tetramethylbutyl)-phenyl-4-fluorobenzylamine, N,N-bis-4-(1,1,3,3-tetramethylbutyl)-phenyl-N- $\beta$ -naphthyl-4-nitrobenzylamine, and N,N-bis-4-(1,1,3,3-tetramethylbutyl)-phenyl-2,2-dimethyl-2-phenylethylamine.

2. The second tertiary amine can be selected from: N-4-(1,1,3,3-tetramethylbutyl)-phenyl-N- $\alpha$ -naphthylbenzylamine, N-4-(1,1,3,3-tetramethylbutyl)-phenyl-N- $\alpha$ -naphthyl-2-phenylethylamine, N-4-(1,1,3,3-tetramethylbutyl)-phenyl-N- $\alpha$ -naphthyl-2-methylbenzylamine, N-4-(1,1,3,3-tetramethylbutyl)-

phenyl-N- $\alpha$ -naphthyl-4-methylbenzylamine, N-4-(1,1,3,3-tetramethylbutyl)-phenyl-N- $\alpha$ -naphthyl-2-chlorobenzylamine, N-4-(1,1,3,3-tetramethylbutyl)-phenyl-N- $\alpha$ -naphthyl-4-chlorobenzylamine, N-4-(1,1,3,3-tetramethylbutyl)-phenyl-N- $\alpha$ -naphthyl-2,4-dichlorobenzylamine, N-4-(1,1,3,3-tetramethylbutyl)-phenyl-N- $\alpha$ -naphthyl-3,4-dichlorobenzylamine, N-4-(1,1,3,3-tetramethylbutyl)-phenyl-N- $\alpha$ -naphthyl- $\alpha$ ,  $\alpha$ -dichloro, benzylamine, N-4-(1,1,3,3-tetramethylbutyl)-phenyl-N- $\alpha$ -naphthyl-2-fluorobenzylamine, N-4-(1,1,3,3-tetramethylbutyl)-phenyl-N- $\alpha$ -naphthyl-4-nitrobenzylamine, and N-4-(1,1,3,3-tetramethylbutyl)-phenyl-N- $\alpha$ -naphthyl-2,2-dimethyl-2-phenylethylamine, or from the following tertiary amines: N-4-(1,1,3,3-tetramethylbutyl)-phenyl-N- $\beta$ -naphthylbenzylamine, N-4-(1,1,3,3-tetramethylbutyl)-phenyl-N- $\beta$ -naphthyl-2-phenylethylamine, N-4-(1,1,3,3-tetramethylbutyl)-phenyl-N- $\beta$ -naphthyl-2-methylbenzylamine, N-4-(1,1,3,3-tetramethylbutyl)-phenyl-N- $\beta$ -naphthyl-4-methylbenzylamine, N-4-(1,1,3,3-tetramethylbutyl)-phenyl-N- $\beta$ -naphthyl-2-chlorobenzylamine, N-4-(1,1,3,3-tetramethylbutyl)-phenyl-N- $\beta$ -naphthyl-4-chlorobenzylamine, N-4-(1,1,3,3-tetramethylbutyl)-phenyl-N- $\beta$ -naphthyl-2,4-dichlorobenzylamine, N-4-(1,1,3,3-tetramethylbutyl)-phenyl-N- $\beta$ -naphthyl-3,4-dichlorobenzylamine, N-4-(1,1,3,3-tetramethylbutyl)-phenyl-N- $\beta$ -naphthyl- $\alpha$ ,  $\alpha$ -dichlorobenzylamine, N-4-(1,1,3,3-tetramethylbutyl)-phenyl-N- $\beta$ -naphthyl-2-fluorobenzylamine, N-4-(1,1,3,3-tetramethylbutyl)-phenyl-N- $\beta$ -naphthyl-4-fluorobenzylamine, N-4-(1,1,3,3-tetramethylbutyl)-phenyl-N- $\beta$ -naphthyl-4-nitrobenzylamine, N-4-(1,1,3,3-tetramethylbutyl)-phenyl-N-1-(1,1,3,3-tetramethylbutyl)- $\beta$ -naphthylbenzylamine, and N-4-(1,1,3,3-tetramethylbutyl)-phenyl-N- $\beta$ -naphthyl-2,2-dimethyl-2-phenylethylamine.

In other preferred embodiments of the embodiments set forth in the above Summary and in Embodiments A and A-1, supra:

1. The lubricant composition contains 0.5-10 parts of a phosphorus-containing ester selected from the group consisting of tricresyl phosphate, triphenyl phosphate, cresyldiphenyl phosphate, xylyldiphenyl phosphate, triethyl phosphate, tributyl phosphate and triisooctyl phosphate.

2. The lubricant composition contains 0-1 part (or 0.002-1 part) 3-amino-1,2,4-triazole, 4-amino-1,2,4-triazole, benzotriazole, 5,5-methylene-bis(1,2,3-benzotriazole), and an alkyl benzotriazole.

3. The carboxylic acid ester component of the lubricant composition is an ester derived from an aliphatic carboxylic acid having 3-18 carbon atoms and a polyol selected from the group consisting of trimethylolpropane, pentaerythritol, dipentaerythritol, tripenterythritol and neopentylglycol.

In another preferred embodiment ("Embodiment B") this invention is directed to:

A lubricant composition comprising:

- a. 100 parts of carboxylic acid ester;
- b. 0.5-10 parts of tricresyl phosphate;
- c. 0.5-8 parts of 4,4'-(1,1,3,3-tetramethylbutyl) di-phenylamine;
- d. 0.5-10 parts of a tertiary amine selected from a group consisting of N,N-bis-4-(1,1,3,3-tetramethylbutyl)-phenyl-N- $\alpha$ -naphthylbenzyl-

- mine, and N-4-(1,1,3,3-tetramethylbutyl)-phenyl- $\beta$ -naphthylbenzylamine; and
- e. 0-0.5 parts of a member selected from a third group consisting of an amino-1,2,4-triazole, benzotriazole, 5,5-methylene-bis-(1,2,3-benzotriazole), and an alkyl benzotriazole in which the alkyl group preferably has 1-12 carbon atoms.

In another preferred embodiment ("Embodiment 'C'") this invention is directed to:

- A lubricant composition comprising:
- 100 parts of a carboxylic acid ester;
  - 0.5-10 parts of tricresyl phosphate;
  - 0.5-8 parts of a secondary amine selected from a first group consisting of N-4-(1,1,3,3-tetramethylbutyl)phenyl- $\alpha$ -naphthylamine, and N-4-(1,1,3,3-tetramethylbutyl)phenyl- $\beta$ -naphthylamine;
  - 0.5-10 parts of N,N-bis-4(1,1,3,3-tetramethylbutyl) phenyl-benzylamine; and
  - 0-0.5 parts of a member selected from a third group consisting of an amino-1,2,4triazole, 5,5-methylene-bis-(1,2,3-benzotriazole), and an alkyl benzotriazole in which the alkyl group preferably has 1-12 carbon atoms.

#### DETAILED DESCRIPTION OF THE INVENTION

It has now been found by practice of the present invention that there is provided a new improved ester base lubricant composition by including a secondary aromatic amine component having two aromatic groups attached to the nitrogen atom and a small amount of alkylated tertiary amine having at least two aromatic groups attached to the nitrogen atom of said amine in the ester base lubricant. In use, the present lubricant composition exhibits improved oxidative stability not only at moderate use temperature, but also at high temperatures (i.e., about 250°F to about 400°F and higher), and metals and related materials lubricated by the composition of this invention often show increased service life, decreased wear, and less corrosion. This lubricant is further advantageously characterized as having decreased sensitivity to form harmful deposits with increasingly excellent lubricating performance under more stringent testing conditions recently adopted by lubricant users. The present composition and method for using said composition offer improved lubricating performance relative to related compositions and methods of the prior art, while providing the art with a means to meet many of the ever increasing lubricant performance requirements of super-sonic jet aircraft and the like.

Generally speaking the present lubricating composition (lubricant composition) includes a major portion of a carboxylic acid ester component having good lubricating (lubricant) qualities, a minor amount of a secondary aromatic amine component and a minor amount of a tertiary aromatic amine component, said amines, being selected according to the teachings of the Summary or Embodiments A and A-1 supra.

Alternatively, the lubricant (lubricating) composition of this invention includes a major portion of a carboxylic acid ester component having good lubricant (lubricating) qualities and a minor amount of each of two tertiary amines as recited in Embodiment A, supra.

The lubricant composition of this invention can include other additives (among such additives are esters

of phosphoric acid, detergents, viscosity index improves, extreme pressure additives, rust inhibitors, and the like which —like carboxylic ester lubricants —are well known in the art).

The carboxylic acid ester component of the present lubricant composition may be almost any carboxylic acid ester having good lubricating qualities. Typically, this ester component is a diester having the general formula  $R_5OOC(CH_2)_nCOOR_6$  wherein  $n$  is an integer from about 2 to about 30 and  $R_5$  and  $R_6$  are members selected from the group consisting of straight and branched chain alkyl groups having from about 6 to about 20 carbon atoms. Preferably,  $n$  is an integer from about 4 to about 8 and  $R_5$  and  $R_6$  are selected from straight and branched chain alkyl groups having 8-16 carbon atoms.

A preferred class of esters from which the carboxylic acid ester component may be selected includes those esters derived from aliphatic monocarboxylic acids by esterifying these acids with polyols, i.e., aliphatic alcohols having 2 or more hydroxy groups. Aliphatic monocarboxylic acids which have from about 3 to about 18, and preferably from about 4 to about 12 carbon atoms are useful. Suitable polyols include, to name a few, trimethylolpropane, pentaerythritol, neopentyl glycol, dipentaerythritol, tripentaerythritol and mixtures thereof. Exemplary esters of this class include pentaerythrityl tetrabutyrate, pentaerythrityl tetracaproate, pentaerythrityl dibutyrate-dicaproate, mixed  $C_4$  to  $C_{10}$  saturated fatty acid esters of pentaerythritol, dipentaerythrityl mixed hexaesters of  $C_4$  to  $C_{10}$  fatty acids, trimethylolpropane trioctanoate and the like.

Another class of esters which may be included in the present lubricant composition are aliphatic polyesters having the following general formula:



Wherein  $R_7$  is an alkyl group having from 1 to about 12 carbon atoms, and preferably from about 5 to about 12 carbon atoms.  $R_8$  is an alkylene group having from about 2 to about 34 carbon atoms in straight or branched chain configuration.  $R_9$  is an alkylene or oxy-alkylene group having from about 2 to about 20 carbon atoms. These polyesters can be prepared, for example, by esterifying two moles of an alkanedioic acid per mole of glycol, followed by esterifying the resulting diester product with two moles of alkanol per mole of the product.

The ester component of the present lubricant composition can include mixtures of the above-described carboxylic acid esters. Typically, the composition includes the ester component in a major amount.

The secondary aromatic amine component of the present lubricant can be selected from those secondary amines having two aromatic groups attached to a nitrogen atom of the amine. The aromatic groups can be heterocyclic or homocyclic, as desired. The aromatic groups of the amine component can have the same or different formulas, as desired. Exemplary of aromatic amines suitable herein are, to name a few, phenyl- $\alpha$ -naphthylamine, diphenylamine, phenyl- $\beta$ -naphthylamine, and preferably the alkyl substituted derivatives of these compounds. Typically, the aromatic groups are identical to each other and include alkyl

groups substituted thereon, preferably in a para position relative to a carbon atom bonded to the amine nitrogen. The alkyl groups can have from about 1 to about 12 carbon atoms and preferably about 8 carbon atoms. A preferred amine component is 4,4'-(1,1,3,3-tetramethylbutyl)-diphenylamine. The secondary amine component of our lubricant can be included in a minor amount such as typically from about 0.5 to about 8 parts by weight, and preferably from about 1 to about 4 parts by weight per 100 parts by weight of the carboxylic acid ester component of said lubricant.

The tertiary amine component of the present lubricant can be represented by the following general formula



wherein R and R<sub>1</sub> are aryl groups and R<sub>2</sub> is an aralkyl group such that at least one of said R, R<sub>1</sub> and R<sub>2</sub> contains an alkyl group having 1-12 carbon atoms.

The tertiary amines used in the lubricating composition of this invention can be prepared in good quantity and in the relatively pure state as disclosed in copending application U.S. Ser. No. 152,372, filed June 11, 1971, now abandoned and assigned to W. R. Grace and Co. when a secondary amine having the formula



where R is an aryl group and R<sub>1</sub> is an aryl group which may be the same as R, is reacted with sodium hydride in the presence of dimethylsulfoxide (DMSO) and the product of this reaction is reacted with an aralkyl halide compound such as benzyl chloride, benzyl bromide, benzyl iodide, 1-bromo-3-phenylpropane, 1-chloro-4-phenyl-n-butane, or the like to form the desired tertiary amine which is recovered. Preferably R and R<sub>1</sub> are aryl groups having 6-12 carbon atoms, at least one group of which contains a halo, nitro, hydroxy, aryl, alkyl or the like group.

The final tertiary amine anti-oxidant which is obtained when an aralkyl halide compound, is reacted with an aromatic secondary amine is represented by the general formula:



wherein R<sub>2</sub> is an aralkyl radical having 7-22 carbon atoms and R and R<sub>1</sub> are separately selected from a group consisting of an aryl group having 6-22 carbon atoms and an alkaryl group having 7-22 carbon atoms such that at least one of R and R<sub>1</sub> is an alkaryl radical having 7-22 carbon atoms. R<sub>2</sub> can contain at least one

of the following: halo, nitro, hydroxy, alkyl alkoxy, aryl, or the like. Preparation of tertiary amines used in the instant invention is described in copending U.S. Pat. application Ser. No. 379,835, filed 7/16/73; which is assigned to W. R. Grace and Co, and which is a continuation-in-part of U.S. Pat. application Ser. No. 152,372, filed June 11, 1972, and now abandoned which is also assigned to W. R. Grace and Co.

The aralkyl halide compound which is used in this invention is preferably benzyl chloride, a substituted benzyl chloride or an aralkyl halide. For example those aralkyl halides having the following general formula are operable:

15

20

25

30

35



wherein n is an integer in the range of 0-6, A, B, F, D, E, G, I, J, K, L, M, and N are members of the group selected from hydrogen, halo, nitro, hydroxy, alkyl, and alkoxy groups, X is either chlorine or bromine, R<sub>3</sub> is either hydrogen or a methyl group and R<sub>4</sub> is either hydrogen or a methyl group. Preferably the alkyl and alkoxy groups have 1-12 carbon atoms.

Some of the tertiary amines which can be prepared and used herein are, more particularly, represented by the following:



55

60

65

wherein R<sub>11</sub>, R<sub>12</sub>, R<sub>13</sub>, and R<sub>14</sub> may be hydrogen, an alkyl or alkoxy groups having 1-12 carbon atoms, an aryl group containing 6-22 carbon atoms, or a halo, nitro, or the like group such that at least one of said R<sub>11</sub>, R<sub>12</sub>, R<sub>13</sub>, and R<sub>14</sub> is said alkyl group, R<sub>15</sub>, R<sub>15'</sub>, R<sub>16</sub>, R<sub>16'</sub>, and R<sub>17</sub> may be hydrogen, an alkyl or alkoxy group having 1-12 carbon atoms, or a halo, nitro, or the like group, n is an integer from 0-6, R<sub>3</sub> is either hydrogen or a methyl group and R<sub>4</sub> is either hydrogen or a methyl group;

13



Wherein  $R_{21}$ ,  $R_{21'}$ ,  $R_{22}$ ,  $R_{22'}$ , and  $R_{23}$  are hydrogen, an alkyl or alkoxy group containing 1-12 carbon atoms, or halo, nitro, or the like groups,  $R_{20}$  is an alkyl or alkoxy group containing 1-12 carbon atoms and  $n$  is an integer from 0-6.  $R_3$  is either hydrogen or a methyl group and  $R_4$  is either hydrogen or a methyl group; and



Where  $R_{31}$ ,  $R_{31'}$ ,  $R_{32}$ ,  $R_{32'}$ , and  $R_{33}$ , are hydrogen, 35  
 an alkyl or alkoxy group having 1-12 carbon atoms, or  
 halo, nitro, or the like groups,  $R_{30}$  is an alkyl or alkoxy  
 group containing 1-12 carbon atoms,  $R_{34}$  is hydrogen, 40  
 an alkyl or alkoxy group containing 1-12 carbon atoms,  
 an aryl group containing 6-10 carbon atoms, or  
 halo, nitro, or the like groups,  $n$  is an integer from 0-6,  
 $R_3$  is either hydrogen or a methyl group and  $R_4$  is either  
 hydrogen or a methyl group. The choice of which sec- 45  
 ondary aromatic amine is to be used is, of course, de-  
 pendent upon which tertiary amine is desired. For ex-  
 ample, to prepare N,N-bis-4-(1,1,3,3 tetramethylbutyl)-  
 phenylbenzylamine, the secondary amine is 4,4'-(1,1,3,3 50  
 tetramethylbutyl)-diphenylamine, and to  
 prepare N,N-bis-4-(2,2,3,3 tetramethylbutyl)phenyl-  
 benzylamine, the secondary amine is 4,4'-(2,2,3,3 tetr-  
 amethylbutyl)-diphenylamine.

Tertiary amines which are especially useful in the lubricating composition of this invention include the following:



**N-4-(1,1,3,3-tetramethylbutyl)-phenyl-N- $\beta$ -naphthylbenzylamine**

14



### N-4-(1,1,3,3-tetramethylbutyl)phenyl N- $\alpha$ -naphthylbenzylamine

- N,N-bis-4-(1,1,3,3-tetramethylbutyl)phenyl-3,4-dichlorobenzylamine,
- N,N-bis-4-(1,1,3,3-tetramethylbutyl)phenyl-2,4-dichlorobenzylamine,
- N,N-bis-4-(1,1,3,3-tetramethylbutyl)phenyl-2-methylbenzylamine,
- N,N-bis-4-(1,1,3,3-tetramethylbutyl)phenyl-2-chlorobenzylamine,
- N,N-bis-4-(1,1,3,3-tetramethylbutyl)phenyl-4-bromobenzylamine,
- N,N-bis-4-(1,1,3,3-tetramethylbutyl)phenyl- $\alpha$ - $\alpha$ -dichlorobenzylamine,
- N,N-bis-4-(1,1,3,3-tetramethylbutyl)phenyl-4-nitrobenzylamine.



### N-4-(2,2,3,3-tetramethylbutyl)-phenyl-N- $\beta$ -naphthylbenzylamine



**N-4-(2,2,3,3-tetramethylbutyl)phenyl-N- $\alpha$ -naphthylbenzylamine**

65 N,N-bis-4-(2,2,3,3-tetramethylbutyl)phenyl-3,4-dichlorobenzylamine,  
N,N-bis-4-(2,2,3,3-tetramethylbutyl)phenyl-2,4-dichlorobenzylamine,

N,N-bis-4-(2,2,3,3-tetramethylbutyl)phenyl-2-methylbenzylamine,  
 N,N-bis-4-(2,2,3,3-tetramethylbutyl)phenyl-2-chlorobenzylamine,  
 N,N-bis-4-(2,2,3,3-tetramethylbutyl)phenyl-4-bromobenzylamine,  
 N,N-bis-4-(2,2,3,3-tetramethylbutyl)phenyl- $\alpha$ - $\alpha$ -dichlorobenzylamine, and  
 N,N-bis-4-(2,2,3,3-tetramethylbutyl)phenyl-4-nitrobenzylamine.

More particularly the process of preparing the tertiary amines used herein which should be followed to obtain optimum results is as follows: dimethylsulfoxide is heated to a temperature of about 60°C. To this is added the sodium hydride. The NaH is preferably added in an amount such that the mole ratio of later added secondary amine to sodium (as Na) added as NaH is about 1:1.1. In many of the examples a 60% by weight dispersion of sodium hydride in mineral oil was used since it is a common way of obtaining sodium hydride commercially. The amount of dimethylsulfoxide used in the reaction is dependent on the molecular weight of the secondary aromatic amine which is used. A 1:1 mole ratio is operable and has produced excellent results, but generally about 0.5 mole excess dimethylsulfoxide is used to assure complete reaction. Following the addition of the sodium hydride the solution generally turns slightly orange with the evolution of hydrogen. After all gas evolution has stopped, the reaction mixture is agitated for sufficient time (about  $\frac{1}{2}$  hour) to attain a complete reaction mixture and the desired secondary aromatic amine is added. Addition of the secondary aromatic amine to the reaction flask normally results in a small exotherm reaction. Therefore, to assure sufficient control of the reaction it is preferable to keep the reaction mixture's temperature below 100°C. by adding the secondary aromatic amine slowly, and cooling if necessary. After adding the secondary amine the reaction mixture is agitated (e.g., stirred) for about 2 hours. The desired aralkyl halide is then added. The mole ratio of secondary aromatic amine to aralkyl halide is also about 1:1. The reaction temperature should not be allowed to exceed 100°C; hence; the aralkyl halide is added slowly. This reaction mixture is then agitated to assure substantial complete reaction (about 6 hours at 90°-100°C) and the reaction is then terminated by adding water cautiously, e.g., dropwise.

The reaction mixture (following addition of the water) is a viscous oil. Toluene is added to the viscous oil to form a workable solution and to this solution NaH-CO<sub>3</sub> is added. Said workable solution is washed with water until substantially neutral. The remaining solvents can be removed under vacuum at about 150°C. The resulting tertiary amine is then cooled to about 100°C and poured into suitable containers for future use. Conversions (one pass yields) by the procedure described herein are about 90-95% of theoretical, and product purity is 96-98%.

However, if the process is deviated from, yield and purity are both noticeably affected. For example, if the secondary aromatic amine is added to the dimethylsulfoxide before the addition of the sodium hydride, the conversion is about 80-85% of theory and product purity is only 78-90%.

The tertiary amine component of our lubricant composition cooperates with the secondary aromatic amine

component of our lubricant composition to impart a significant portion of the improved oxidative stability of the present lubricant composition. The tertiary amine component can be included in the composition in an amount from about 0.5 to about 10 parts by weight, and preferably from about 0.5 to about 4 parts by weight based on 100 parts by weight of the carboxylic acid ester component.

The advantageous, although optional triazole component of the present lubricant is an amino substituted triazole compound, and can be selected from 3-amino- and 4-amino-1,2,4-triazole, 5,5-methylene-bis-(1,2,3-benzotriazole), or alternate corrosion inhibitors such as 1,2,3-benzotriazole or alkyl substituted 1,2,3-benzotriazoles. The triazole component can be included in the present composition in an amount of from 0.002 to about 1 part by weight, and preferably from about 0.01 to about 0.2 part by weight based on 100 parts by weight of the carboxylic acid ester component.

20 The preferred amount of triazole is limited only by additive solubility and the user's requirements.

The advantageously, although optionally, included phosphorus-containing acid ester component can be selected from triesters of phosphoric acid with alcohols such as straight and branched chain aliphatic alcohols having from 1 to about 8 carbon atoms. Exemplary of these esters are triethyl phosphate, tributyl phosphate and triisooctyl phosphate. Other suitable phosphoric acid esters include esters of phenol, cresols, and naphthols, and the like, these esters can have from 1 to about 3 C<sub>1</sub> to C<sub>10</sub> alkyl substituents on one or more of the aryl moieties. Exemplary of these esters are tricresyl phosphate, triphenyl phosphate, cresyldiphenyl phosphate, xylodiphenyl phosphate, and the like.

The phosphorus-containing acid ester component may be included in an amount from 0 to about 10 parts by weight, and preferably from about 0.5 to about 5 parts by weight per 100 parts by weight of the carboxylic acid ester component.

40 The present lubricant composition can further include metal deactivating agents, anti-corrosion agents, anti-rusting agents, anti-foaming agents, dyes, thickening agents, additional anti-oxidants and other suitable agents known in the art for use in ester-containing lubricants.

We have found that; (a) the amount of amines present in the improved ester base lubricants of our invention is not critical and a finite amount of the amines produces a finite improvement in the oxidative stability of the lubricants; and (b) this is true whether the amines are; (i) a secondary amine and a tertiary amine selected as recited in the Summary or Embodiment A-1, supra; or (ii) two tertiary amines selected as recited in Embodiment A, supra.

55 The present invention will be further illustrated by the following non-limiting examples.

Examples 1-37 describe the preparation of the tertiary amine component of this invention.

#### EXAMPLE 1

To a reaction flask (4-neck, 3 liter flask equipped with a condenser, stirrer, N<sub>2</sub> inlet, thermometer and dropping funnel) containing 1.5 moles of dimethylsulfoxide (DMSO) which had been heated to about 60°C was added 1.1 mole of a 60% by weight dispersion of sodium hydride in mineral oil. The solution was observed to turn slightly orange as the sodium hydride

was added. After all hydrogen evolution had stopped, the reaction mixture was stirred for one-half hour and then 1 mole 4,4'-(1,1,3,3-tetramethylbutyl)-diphenylamine was added to the reaction flask dropwise. The reaction mass was stirred for about 2 hours following which 1 mole of benzyl chloride was added dropwise using a dropping funnel. The reaction temperature was thereby maintained between 60°-70°C. Following addition of the benzyl halide the reaction mixture was stirred for 6 hours at a temperature of 60°-70°C. 200 ml. of water was cautiously added drop-

tetramethyl)-diphenylamine and the product tertiary amine was N,N-bis-4-(2,2,3,3-tetramethylbutyl)-phenylbenzylamine.

5

## Examples 2-9

Examples 2 through 9 followed the procedure of Example 1 except that the appropriate benzyl compound was added to the 4,4'-(1,1,3,3-tetramethylbutyl)-diphenylamine in order to prepare the tertiary amine derivatives shown in Table 1.

Table 1

| Example No. | Benzyl Compound Used        | Tertiary Amine Obtained                                                   |
|-------------|-----------------------------|---------------------------------------------------------------------------|
| 2           | 3,4-dichlorobenzyl chloride | N,N-bis-4-(1,1,3,3-tetramethylbutyl)phenyl-3,4-dichlorobenzylamine        |
| 3           | 2,4-dichlorobenzyl chloride | N,N-bis-4-(1,1,3,3-tetramethylbutyl)phenyl-2,4-dichlorobenzylamine        |
| 4           | 2-methylbenzyl chloride     | N,N-bis-4-(1,1,3,3-tetramethylbutyl)phenyl-2-methylbenzylamine            |
| 5           | 2-chlorobenzyl chloride     | N,N-bis-4-(1,1,3,3-tetramethylbutyl)phenyl-2-chlorobenzylamine            |
| 6           | 4-bromobenzyl bromide       | N,N-bis-4-(1,1,3,3-tetramethylbutyl)phenyl-4-bromobenzylamine             |
| 7           | 2-ethylbenzyl chloride      | N,N-bis-4-(1,1,3,3-tetramethylbutyl)phenyl-2-ethylbenzylamine             |
| 8           | benzotrichloride            | N,N-bis-4-(1,1,3,3-tetramethylbutyl)phenyl- $\alpha$ -dichlorobenzylamine |
| 9           | 4-nitrobenzyl chloride      | N,N-bis-4-(1,1,3,3-tetramethylbutyl)phenyl-4-nitrobenzylamine             |

wise to terminate the reaction. The viscous oil in the reaction flask was then extracted with 400 ml. of toluene and washed once with 200 ml. of a 10% by weight NaHCO<sub>3</sub> solution. The solution was washed several more times with 200 ml. aliquots of water until the washings were neutral. The remaining solvents and volatiles were removed under vacuum at 65°C. The result-

30

Examples 2 through 9 followed the procedure of Example 1A except that the appropriate benzyl compound was added to the 4,4'-(2,2,3,3-tetramethylbutyl)-diphenylamine in order to prepare the tertiary amine derivatives shown in Table 1A.

Table 1-A

| Example No. | Benzyl Compound Used        | Tertiary Amine Obtained                                                   |
|-------------|-----------------------------|---------------------------------------------------------------------------|
| 2           | 3,4-dichlorobenzyl chloride | N,N-bis-4-(2,2,3,3-tetramethylbutyl)phenyl-3,4-dichlorobenzylamine        |
| 3           | 2,4-dichlorobenzyl chloride | N,N-bis-4-(2,2,3,3-tetramethylbutyl)phenyl-2,4-dichlorobenzylamine        |
| 4           | 2-methylbenzyl chloride     | N,N-bis-4-(2,2,3,3-tetramethylbutyl)phenyl-2-methylbenzylamine            |
| 5           | 2-chlorobenzyl chloride     | N,N-bis-4-(2,2,3,3-tetramethylbutyl)phenyl-2-chlorobenzylamine            |
| 6           | 4-bromobenzyl bromide       | N,N-bis-4-(2,2,3,3-tetramethylbutyl)phenyl-4-bromobenzylamine             |
| 7           | 2-ethylbenzyl chloride      | N,N-bis-4-(2,2,3,3-tetramethylbutyl)phenyl-2-ethylbenzylamine             |
| 8           | benzotrichloride            | N,N-bis-4-(2,2,3,3-tetramethylbutyl)phenyl- $\alpha$ -dichlorobenzylamine |
| 9           | 4-nitrobenzyl chloride      | N,N-bis-4-(2,2,3,3-tetramethylbutyl)phenyl-4-nitrobenzylamine             |

ing tertiary amine was cooled to 38°C and poured into a suitable container. The yield of the resulting tertiary amine was 90% of the theoretical value and had a purity of about 98%. The structure of the tertiary amine was determined by infrared spectroscopy and nuclear magnetic resonance spectroscopy to be N,N-bis-4-(1,1,3,3-tetramethylbutyl)-phenyl-benzylamine. Product purity was determined by infrared spectroscopy and thin layer chromatography.

55

Examples 1-9 were repeated except that 1 mole of N-4-(1,1,3,3-tetramethylbutyl)-phenyl- $\alpha$ -naphthylamine was substituted for the 1 mole of 4,4'-(1,1,3,3-tetramethylbutyl)-diphenylamine. In each example the appropriate tertiary amine was obtained in good yield and at high purity.

## Example 1A

The general procedure of Example 1, was repeated; however, in this instance the 4,4'-(1,1,3,3-tetramethylbutyl)-diphenylamine was replaced with 4,4'-(2,2,3,3-

65

Examples 1-9 were repeated except that 1 mole of N-4-(1,1,3,3-tetramethylbutyl)-phenyl- $\alpha$ -naphthylamine was substituted for the 1 mole of 4,4'-(1,1,3,3-tetramethylbutyl)-diphenylamine. In each example the appropriate tertiary amine was obtained in good yield and at high purity.

## Examples 10-18

Examples 10-18

Examples 1-9 were repeated except that 1 mole of N-4-(1,1,3,3-tetramethylbutyl)-phenyl- $\alpha$ -naphthylamine was substituted for the 1 mole of 4,4'-(1,1,3,3-tetramethylbutyl)-diphenylamine. In each example the appropriate tertiary amine was obtained in good yield and at high purity.

## Examples 19-27

Examples 19-27

Examples 1-9 were repeated except that 1 mole of N-4-(1,1,3,3-tetramethylbutyl)-phenyl- $\alpha$ -naphthylamine was substituted for the 1 mole of 4,4'-(1,1,3,3-tetramethylbutyl)-diphenylamine. In each example the appropriate tertiary amine was obtained in good yield and at high purity.

## Examples 28-36

Example 1 was repeated except that 1 mole of N-4-(1,1,3,3-tetramethylbutyl)phenyl- $\beta$ -( $\alpha$ -propyl)-naphthylamine was substituted for the 1 mole of 4,4'-(1,1,3,3-tetramethylbutyl)-diphenylamine. In each example the appropriate tertiary amine was obtained in good yield and at high purity.

## Example 37

The procedure of Example 1 was followed except that 2,2-dimethyl-2-phenylethyl chloride was used in place of benzyl chloride. The appropriate tertiary amine was obtained in good yield and high purity.

## Examples 38-46

Examples 38-46 illustrate the effect of a 400°F 72 Hour Corrosion Oxidation Test on prior art ester base lubricants compositions.

In said test a 0.032 inch  $\times$  1 inch  $\times$  1 inch metal test specimen is placed in a glass tube and 100 ml of a liquid lubricant composition to be tested is placed in the glass tube to cover the test specimen, and the sample (test specimen plus composition to be tested) is heated to and maintained at a substantially constant temperature of about 400°C while passing 5 liters of clean dry air through the lubricant composition for 72 hours.

The metals used in these tests included magnesium, aluminum, iron, copper and electrolytic grade silver. At the end of a 72 hour testing period, the air flow was terminated and the metal test squares were removed from the compositions, washed in 135°F 1,1,1-trichloroethane, air dried, and thereafter weighed. Metal weight changes from before to after testing, ex-

protective coating which is occasionally formed on the individual test specimens.

The test included also measuring kinematic viscosity at 100°F of the various compositions tested, before and after testing, using the procedure of ASTM Standard D 445. The results are given below in Table 2 as percent increase in viscosity. Acid value changes (the difference in acid value after and before running the 72 Hour Corrosion Oxidation Test) were also run on each lubricant composition tested. The acid value changes are also shown in Table 2. The acid values used for calculating the changes were measured by potentiometric titration with potassium hydroxide to an end point of pH 11 using the procedure of ASTM Standard D 664. The compositions were observed and rated for sludge content at the end of the 72 Hour Oxidation Corrosion Tests. A sludge rating of nil means essentially no sludge was observed, ratings of light, moderate, heavy, etc. were assigned for increasing amounts of observed sludge.

In each of Examples 38-42 the composition tested comprised an ester base lubricant component, a secondary aromatic amine, a phosphorus-containing ester, and an amino substituted, 1,2,4-triazole component. Each composition is unacceptable because of a high acid number change, a viscosity change, or a presence of sludge. Acceptable values are as follows:

|                      |             |
|----------------------|-------------|
| Acid No. Change      | 2.0 or less |
| Viscosity Change     | 25% or less |
| Visual Sludge Rating | Nil         |

In Examples 43-46 the composition contained two different secondary amines. Although improved results (as compared with Examples 38-42) were obtained, the compositions used in Examples 43-46 were also unacceptable because of sludge formation.

Table 2

| COMPOSITION<br>Example No.                                     | RESULTS OF 400°F, 72 HOUR CORROSION-OXIDATION TESTS <sup>a</sup><br>PARTS BY WEIGHT |        |        |          |        |        |        |        |        |
|----------------------------------------------------------------|-------------------------------------------------------------------------------------|--------|--------|----------|--------|--------|--------|--------|--------|
|                                                                | 38                                                                                  | 39     | 40     | 41       | 42     | 43     | 44     | 45     | 46     |
| Carboxylic Acid Ester <sup>b</sup>                             | 100                                                                                 | 100    | 100    | 100      | 100    | 100    | 100    | 100    | 100    |
| Phenyl- $\alpha$ -naphthylamine                                | 1.0                                                                                 |        |        |          |        |        |        |        |        |
| Phenyl- $\beta$ -naphthylamine                                 |                                                                                     | 1.0    |        |          |        |        |        |        |        |
| 4,4'-(1,1,3,3-tetramethylbutyl)-diphenylamine                  |                                                                                     |        | 2.0    |          |        | 2.0    | 2.0    | 2.0    | 2.0    |
| N-4-(1,1,3,3-tetramethylbutyl)-phenyl- $\alpha$ -naphthylamine |                                                                                     |        |        | 1.5      |        |        |        | 1.5    |        |
| N-4-(1,1,3,3-tetramethylbutyl)-phenyl- $\beta$ -naphthylamine  |                                                                                     |        |        |          | 1.5    |        |        |        | 1.5    |
| Tricresyl phosphate                                            | 1.0                                                                                 | 1.0    | 1.0    | 1.0      | 1.0    | 1.0    | 1.0    | 1.0    | 1.0    |
| 3-amino-1,2,4-triazole                                         | 0.05                                                                                | 0.05   | 0.05   | 0.05     | 0.05   | 0.05   | 0.05   | 0.05   | 0.05   |
| Corrosion, mg/cm <sup>2</sup>                                  |                                                                                     |        |        |          |        |        |        |        |        |
| Magnesium                                                      | 0.000                                                                               | -0.010 | -0.405 | -0.023   | -0.117 | -0.039 | -0.085 | +0.031 | -0.023 |
| Aluminum                                                       | -0.015                                                                              | +0.010 | +0.015 | -0.023   | -0.101 | -0.023 | -0.039 | +0.015 | -0.031 |
| Copper                                                         | -0.031                                                                              | -0.046 | -0.010 | -0.039   | -0.046 | -0.078 | -0.039 | -0.023 | -0.070 |
| Iron                                                           | -0.015                                                                              | +0.010 | +0.023 | -0.023   | -0.078 | -0.015 | -0.023 | +0.015 | -0.010 |
| Silver                                                         | -0.031                                                                              | -0.010 | -0.023 | -0.054   | -0.062 | -0.163 | -0.078 | +0.015 | -0.054 |
| Total Acid No. Change, mg KOH/g                                | 2.50                                                                                | 5.50   | 8.20   | 1.14     | 3.67   | 0.65   | 0.72   | 0.57   | 0.72   |
| Viscosity Change (100°F), %                                    | 24.8                                                                                | 40.0   | 44.8   | 14.2     | 36.0   | 19.0   | 18.3   | 18.0   | 18.6   |
| Visual Sludge Rating                                           | Heavy                                                                               | Heavy  | Heavy  | Moderate | Moder. | Moder. | Moder. | Light  | Light  |

<sup>a</sup>The compositions tested in Examples 38-46 and reported in this table are prior art compositions—not the compositions of this invention.

<sup>b</sup>A technical pentaerythritol ester made from C<sub>6</sub>, C<sub>7</sub> and C<sub>8</sub> straight chain monocarboxylic acids.

pressed in milligrams per square centimeter of metal surface, are shown below in Table 2 for various lubricant compositions. The "+" figures are caused by a

65 The following examples show the effect of using an alkylated tertiary amine as part of the lubricant composition to improve stability and resistance to oxidation.

## Examples 47-60

The compositions prepared as shown in Table 3 were subjected to the 400°F., 72 Hour Corrosion Oxidation

Examples 47-60 are summarized in Table 3. Results shown in this table illustrate the improvement obtained with the additives of this invention.

TABLE 3  
Results of 400° F., 72 hour corrosion-oxidation tests <sup>a</sup>

| Example number                                                         | Parts by weight |        |        |        |        |        |        |        |        |        |        |        |        |        |
|------------------------------------------------------------------------|-----------------|--------|--------|--------|--------|--------|--------|--------|--------|--------|--------|--------|--------|--------|
|                                                                        | 47              | 48     | 49     | 50     | 51     | 52     | 53     | 54     | 55     | 56     | 57     | 58     | 59     | 60     |
| <b>Composition:</b>                                                    |                 |        |        |        |        |        |        |        |        |        |        |        |        |        |
| Carboxylic acid ester <sup>b</sup>                                     | 100             | 100    | 100    | 100    | 100    | 100    | 100    | 100    | 100    | 100    | 100    | 100    | 100    | 100    |
| N-4-(1,1,3,3-tetramethylbutyl)-phenyl-N- $\alpha$ -naphthylbenzylamine | 1.9             |        |        |        |        |        |        |        |        |        | 1.9    |        | 1.9    |        |
| N-4-(1,1,3,3-tetramethylbutyl)-phenyl-N- $\beta$ -naphthylbenzylamine  |                 | 1.9    |        |        |        |        |        |        |        |        | 1.9    |        | 1.9    |        |
| N,N-bis-4-(1,1,3,3-tetramethylbutyl)-phenylbenzylamine                 |                 |        | 2.5    |        | 2.5    | 2.5    |        |        |        |        | 1.9    |        | 1.9    |        |
| N,N-bis-4-(1,1,3,3-tetramethylbutyl)-phenyl-2-phenylethylamine         |                 |        |        | 2.6    |        |        | 2.6    | 2.6    |        |        | 2.6    | 2.6    |        | 2.5    |
| 4,4'-(1,1,3,3-tetramethylbutyl)-diphenylamine                          |                 |        |        |        |        |        |        |        | 2.0    | 2.0    |        |        |        |        |
| N-4-(1,1,3,3-tetramethylbutyl)-phenyl- $\alpha$ -naphthylamine         |                 |        |        |        | 1.5    |        | 1.5    |        |        |        |        |        |        |        |
| N-4-(1,1,3,3-tetramethylbutyl)-phenyl- $\beta$ -naphthylamine          |                 |        |        |        |        |        |        |        |        |        |        |        |        |        |
| Tricresyl phosphate                                                    | 1.0             | 1.0    | 1.0    | 1.0    | 1.0    | 1.0    | 1.0    | 1.0    | 1.0    | 1.0    | 1.0    | 1.0    | 1.0    | 1.0    |
| 3-amino-1,2,4-triazole                                                 | 0.05            | 0.05   | 0.05   | 0.05   | 0.05   | 0.05   | 0.05   | 0.05   | 0.05   | 0.05   | 0.05   | 0.05   | 0.05   | 0.05   |
| <b>Corrosion, mg./cm.<sup>2</sup>:</b>                                 |                 |        |        |        |        |        |        |        |        |        |        |        |        |        |
| Magnesium                                                              | +0.023          | -0.015 | 0.000  | -0.015 | -0.032 | +0.039 | +0.015 | +0.015 | -0.031 | +0.010 | +0.023 | +0.046 | 0.000  | +0.015 |
| Aluminum                                                               | -0.015          | -0.031 | -0.015 | -0.023 | +0.015 | -0.010 | -0.000 | 0.010  | +0.010 | 0.000  | -0.010 | +0.010 | -0.010 |        |
| Copper                                                                 | -0.101          | -0.109 | -0.225 | -0.039 | -0.054 | -0.089 | -0.010 | -0.081 | -0.054 | -0.052 | -0.210 | -0.132 | -0.078 | -0.023 |
| Iron                                                                   | +0.015          | -0.010 | +0.023 | -0.015 | +0.015 | +0.010 | -0.010 | 0.000  | +0.028 | +0.054 | +0.039 | +0.023 | +0.023 | +0.062 |
| Silver                                                                 | -0.089          | -0.081 | -0.089 | -0.029 | -0.023 | -0.023 | +0.039 | -0.010 | -0.031 | -0.015 | -0.010 | -0.023 | -0.010 | -0.015 |
| Total acid No. change, mg./KOH/g.                                      | 7.50            | 8.00   | 5.50   | 7.00   | 0.66   | 1.07   | 1.20   | 1.40   | 1.06   | 0.89   | 0.90   | 1.20   | 1.20   | 1.70   |
| Viscosity change (100° F.), percent                                    | 38.3            | 36.7   | 34.9   | 64.7   | 18.6   | 19.7   | 22.1   | 21.8   | 19.0   | 18.0   | 20.1   | 22.1   | 18.8   | 23.6   |
| Visual sludge rating                                                   | Light           | L      | L      | L      | Nil    | N      | N      | N      | N      | N      | N      | N      | N      | N      |

<sup>a</sup> The composition of Examples 51-60 are compositions of the instant invention.

<sup>b</sup> A technical pentaerythritol ester made from C<sub>5</sub>, C<sub>7</sub>, and C<sub>9</sub> straight chain monocarboxylic acids.

## Test described in Examples 38-46.

The ester base lubricant used in Examples 47-60 was a technical pentaerythritol ester made from C<sub>5</sub>, C<sub>7</sub>, and C<sub>9</sub> straight chain alcanoic acids. Said ester was from the same lot that was used in Examples 38-46.

The compositions tested in Examples 47-50 were the ester base lubricant plus the following additives; (a) one tertiary amine; (b) a phosphorus containing ester; and (c) a 1,2,4-triazole component. Although sludge formation was light (L), the acid number and viscosity changes were such that these lubricant compositions (those tested in Examples 48-50) were unacceptable.

In Examples 51-56 various secondary aromatic amines were added to the compositions of Examples 47-50 so that the lubricant composition now contained both a secondary amine and an alkylated tertiary amine. In each example the sludge formed was nill (N), and improved, acceptable acid numbers and viscosity changes were obtained.

In Examples 57-60 the lubricant composition contained no secondary amine, but two alkylated tertiary amines. Acceptable results were obtained in each of these examples.

45 When N,N-bis-4-(1,1,3,3-tetramethylbutyl)phenyl-2-phenylethylamine is used in the composition, results obtained show an acid number change<sup>1</sup> of 7.0, a viscosity increase<sup>2</sup> of 64.7%, and sludge formation (Example 50, Table 3). When the additive is a secondary amine,

50 N-4-(1,1,3,3-tetra-methylbutyl)phenyl- $\beta$ -naphthylamine (Example 42, Table 2), the acid number change is 3.67, the viscosity increase is 36.0%, and there is sludge formation. However, combining these two additives in the same lubricating composition (Example 54, Table 3) gives an acid number change of only 1.40 and a 21.8% increase in viscosity, and no evidence of sludge.

<sup>1</sup> The change in the acidity of the composition being tested before and after the 72 Hour Corrosion Oxidation Test measured by potentiometric titration with potassium hydroxide to an end point of pH 11 using the procedure of ASTM Standard D664.

<sup>2</sup> The increase in viscosity as determined by measuring the viscosity of the composition before the 72 Hour Corrosion Oxidation Test and then after said test using the procedure of ASTM Standard D445.

It has also been found that results superior to those attained heretofore are obtained when two different tertiary amines are added to the base stock (carboxylic acid ester lubricant) instead of a secondary and a tertiary amine.

Generally, as shown in Table 3, results of the 72 Hour Corrosion Oxidation Tests show that when two alkylated tertiary amines are used to prepare the composition (Examples 57, 58, 59 and 60), there is a marked reduction in sludge formation and an obvious improvement in oxidation stability.

#### Examples 61-64

In Examples 61-64 Alcor deposition tests of various ester base lubricant compositions with the antioxidants of Table 3 are shown. These tests were conducted to show the effectiveness of the additives in controlling oxidation stability and deposition (cleanliness). In each example 100 parts by weight of a typical lubricant ester base stock and 1 part by weight of a phosphorus-containing ester (tricresyl phosphate) were used. In Example 61 the additive was a secondary amine; in Example 62 the additive was an alkylated secondary amine; in Example 63 the additive was an alkylated tertiary amine; and in Example 64 the additive was a combination of two alkylated tertiary amines.

In Examples 61-64 the compositions described were submitted to the "Alcor High Temperature Deposition Tests". In this test, the purpose of which is to determine cleanliness and oxidation stability of the lubricant being tested, the following test procedure is used. The lubricating composition being tested is circulated through an Alcor Deposition Tester, Model HTDT 1003, manufactured by Alcor, Inc., of San Antonio, Tex. at 300 ml/min. by a high temperature pump. Constant flow is maintained by a constant speed drive. The composition is then heated to a specified temperatures, in this instance 500°F. Any sludge which is formed is

collected on a filter screen and weighed. Ideally, the deposits would be nil, however, the results shown for Examples 63 and 64 are quite acceptable. There is also a formation of deposits on the tube which is being heated. Heat was supplied by an electric current passed through the metal tube. The composition being tested is circulated past the heated tube. The deposits are recognized under the "Tube Deposit Weight." The "Visual Tube Evaluation" is determined by assigning demerits to the composition being tested according to the type of deposit which has formed on the tube. The tube is divided into for example, a flaked carbon deposit over a portion of the tube receives a demerit rating of 20. The demerit rating is then multiplied by the deposit weight per unit length. The deposit weight per unit length is determined by stripping the tube one inch at a time until the full length (10 inches) has been stripped. The total demerit rating is the sum of all ratings divided by 10 and is reported as visual tube evaluation. The demerit values assigned as according to the type of deposit are given in Table 7. The overall rating is the tube deposit weight plus the visual tube evaluation plus the filter screen deposits, all divided by two. An acceptable overall rating is less than 80, and preferably less than 60. Nevertheless, the composition of Example 63 is unsatisfactory because of the high acid number and the high viscosity change. The results of the Alcor High-Temperature Deposition Tests are given in Table 4. Also given are the Acid No. Change (as described heretofore). Clearly the only acceptable composition reported in Table 4 is that of Example 64 which contained two alkylated tertiary amines. The others, Examples 61, 62, and 63 failed the test.

Table 4

| Composition                                                           | Results of Alcor High Temperature Deposition Tests <sup>a</sup> |                  |                  |                  |
|-----------------------------------------------------------------------|-----------------------------------------------------------------|------------------|------------------|------------------|
|                                                                       | 61                                                              | 62               | 63               | 64               |
| Example No.                                                           |                                                                 |                  |                  |                  |
| Carboxylic Acid Ester <sup>b</sup>                                    | 100                                                             | 100              | 100              | 100              |
| Phenyl- $\beta$ -naphthylamine                                        | 1.0                                                             |                  |                  |                  |
| 4-(1,1,3,3-tetramethylbutyl)                                          |                                                                 | 1.5              |                  |                  |
| Phenyl- $\beta$ -naphthylamine                                        |                                                                 |                  |                  |                  |
| N-4-(1,1,3,3-tetramethylbutyl)-phenyl-N- $\beta$ -naphthylbenzylamine |                                                                 |                  | 1.9              | 1.9              |
| N,N-bis-4-(1,1,3,3-tetramethylbutyl)-phenylbenzylamine                |                                                                 |                  |                  | 2.5 <sup>c</sup> |
| Tricresyl phosphate                                                   | 1.0                                                             | 1.0              | 1.0              | 1.0              |
| Test Temperature, °F.                                                 | 550 <sup>d</sup>                                                | 550 <sup>d</sup> | 550 <sup>d</sup> | 550 <sup>d</sup> |
| Tube Deposit Weight, Mg.                                              | 398.5                                                           | 18.6             | 22.0             | 16.0             |
| Visual Tube Evaluation                                                | 140.0                                                           | 133.1            | 58.0             | 26.8             |
| Filter Screen Deposits, Mg.                                           | 39.3                                                            | 62.7             | 22.4             | 19.2             |
| Overall Rating (Cleanliness)                                          | 288.9                                                           | 107.2            | 51.2             | 31.0             |
| Acid No. Change, mg KOH/g                                             | 8.9                                                             | 12.2             | 13.2             | 1.15             |
| Viscosity Change (100°F.), %                                          | 172                                                             | 334              | 62.0             | 14.5             |

<sup>a</sup>The composition of Example 64 is a composition of the instant invention.

<sup>b</sup>A technical pentaerythritol ester made from C<sub>6</sub>, C<sub>7</sub>, and C<sub>8</sub> straight chain monocarboxylic acids.

TABLE 5

| COMPOSITION<br>Example No.                                         | 60 <sup>(1)</sup> | 65   | 66   | 56 <sup>(1)</sup> | PARTS BY WEIGHT |     |                   |     |     |
|--------------------------------------------------------------------|-------------------|------|------|-------------------|-----------------|-----|-------------------|-----|-----|
|                                                                    |                   |      |      |                   | 67              | 68  | 52 <sup>(1)</sup> | 69  | 70  |
| Carboxylic Acid Ester <sup>(2)</sup>                               | 100               | 100  | 100  | 100               | 100             | 100 | 100               | 100 | 100 |
| N-4-(1,1,3,3-tetramethylbutyl)phenyl- $\beta$ -naphthylbenzylamine | 1.9               | 4.4  |      | 1.9               | 3.9             |     |                   |     |     |
| N-4-(1,1,3,3-tetramethylbutyl)phenyl- $\beta$ -naphthylamine       |                   |      |      |                   |                 |     | 1.5               | 4.0 |     |
| N,N-bis-4-(1,1,3,3-tetramethylbutyl)-phenylbenzylamine             | 2.5               |      | 4.4  |                   |                 |     | 2.5               |     | 4.0 |
| 4,4'-(1,1,3,3-tetramethylbutyl)-diphenylamine                      |                   |      |      |                   | 2.0             |     | 3.9               |     |     |
| Tricresyl phosphate                                                | 1.0               | 1.0  | 1.0  | 1.0               | 1.0             | 1.0 | 1.0               | 1.0 | 1.0 |
| 3-amino-1,2,4-triazole                                             | 0.05              | 0.05 | 0.05 | 0.05              | 0.05            | 0.5 | 0.5               | 0.5 | 0.5 |

TABLE 5—Continued

| COMPOSITION<br>Example No.      | PARTS BY WEIGHT   |          |          |                   |          |          |                   |        |          |
|---------------------------------|-------------------|----------|----------|-------------------|----------|----------|-------------------|--------|----------|
|                                 | 60 <sup>(1)</sup> | 65       | 66       | 56 <sup>(1)</sup> | 67       | 68       | 52 <sup>(1)</sup> | 69     | 70       |
| Corrosion, mg/cm <sup>2</sup>   |                   |          |          |                   |          |          |                   |        |          |
| Magnesium                       | +0.015            | -0.023   | -0.007   | +0.010            | -0.015   | -0.015   | +0.039            | +0.015 | +0.015   |
| Aluminum                        | -0.010            | 0.000    | 0.000    | +0.010            | 0.000    | 0.000    | -0.015            | 0.000  | 0.000    |
| Copper                          | -0.023            | -0.078   | -0.078   | -0.052            | -0.109   | -0.093   | -0.039            | -0.046 | -0.132   |
| Iron                            | +0.062            | +0.023   | 0.000    | +0.054            | 0.000    | 0.000    | +0.010            | +0.023 | -0.023   |
| Silver                          | -0.015            | -0.039   | -0.031   | -0.010            | -0.015   | -0.015   | -0.023            | -0.031 | -0.023   |
| Total Acid No. Change, mg KOH/g | 1.70              | 1.54     | 2.96     | 0.90              | 2.20     | 4.1      | 1.07              | 0.69   | 2.81     |
| Viscosity Change (100°F), %     | 23.6              | 21.9     | 44.3     | 20.1              | 20.6     | 37.4     | 19.7              | 17.2   | 40.6     |
| Visual Sludge Rating            | Nil               | Moderate | Moderate | Nil               | Moderate | Moderate | Nil               | Heavy  | Moderate |

<sup>(1)</sup>Data shown were taken from Table 3.<sup>(2)</sup>A technical pentaerythritol ester made from C<sub>5</sub>, C<sub>7</sub>, and C<sub>9</sub> straight chain monocarboxylic acids.

TABLE 6

| COMPOSITION<br>Example No.                                    | 61 <sup>(1)</sup> | 62 <sup>(1)</sup> | 71    | 63   | 72   | 73    | 74   | 64 <sup>(1)</sup> |
|---------------------------------------------------------------|-------------------|-------------------|-------|------|------|-------|------|-------------------|
| Carboxylic Acid Ester <sup>(2)</sup>                          | 100               | 100               | 100   | 100  | 100  | 100   | 100  | 100               |
| Phenyl-β-naphthylamine                                        | 1.0               |                   |       |      |      |       |      |                   |
| N-4-(1,1,3,3-tetramethylbutyl)-phenyl-β-naphthylamine         |                   | 1.5               |       |      |      |       | 1.5  |                   |
| 4,4'-(1,1,3,3-tetramethylbutyl)-diphenylamine                 |                   |                   | 2.0   |      |      |       | 2.0  | 2.0               |
| N-4-(1,1,3,3-tetramethylbutyl)-phenyl-N-β-naphthylbenzylamine |                   |                   |       | 1.9  |      |       | 1.9  | 1.9               |
| N,N-bis-(1,1,3,3-tetramethylbutyl)-phenylbenzylamine          |                   |                   |       |      | 2.5  |       |      |                   |
| Tricresyl phosphate                                           | 1.0               | 1.0               | 1.0   | 1.0  | 1.0  | 1.0   | 1.0  | 2.5               |
| Test Temperature, °F                                          | 550               | 550               | 550   | 550  | 550  | 550   | 550  | 550               |
| Tube Deposits Weight, mg                                      | 398.5             | 18.6              | 90.9  | 22.0 | 24.9 | 32.0  | 40.6 | 16.0              |
| Tube Deposit Rating                                           | 140.0             | 133.1             | 86.6  | 58.0 | 70.0 | 105.9 | 66.6 | 26.8              |
| Filter Screen Deposits, mg                                    | 39.3              | 62.7              | 59.2  | 22.4 | 21.8 | 23.2  | 14.2 | 19.2              |
| Overall Deposit Rating (Cleanliness)                          | 288.9             | 107.2             | 118.3 | 51.2 | 58.3 | 80.5  | 60.7 | 31.0              |
| Acid No. Change, mg KOH/g                                     | 8.9               | 12.2              | 7.9   | 13.2 | 8.2  | 2.4   | 1.01 | 1.15              |
| Viscosity Change (100°F), %                                   | 172               | 334               | 213   | 62.0 | 419  | 97.5  | 40.3 | 14.5              |

<sup>(1)</sup>Data shown were taken from Table 4.<sup>(2)</sup>A technical pentaerythritol ester made from C<sub>5</sub>, C<sub>7</sub>, and C<sub>9</sub> straight chain monocarboxylic acids.

Table 7

| DEPOSIT DESCRIPTION AND DEMERIT VALUES USED FOR NUMERICALLY DESCRIBING DEPOSITS |          |                                                                      |                |
|---------------------------------------------------------------------------------|----------|----------------------------------------------------------------------|----------------|
| Type of Deposit                                                                 | Degree   | Description                                                          | Demerit Rating |
| Flaked Carbon                                                                   | —        | Carbonaceous coating that cannot be removed by wiping with a rag.    | 20             |
|                                                                                 | Heavy    | Broken blisters, peeling.                                            |                |
|                                                                                 | Moderate | Over 3/64-inch in thickness.                                         |                |
|                                                                                 | Light    | Ranges from 1/64-inch to less than 3/64-inch in thickness.           |                |
| Blistered Carbon                                                                | —        | Ranges from just covering to less than 1/64-inch in thickness.       |                |
|                                                                                 | Heavy    | Same as for flaked carbon, blistered, bubbled.                       | 17             |
|                                                                                 | Moderate | Same as for flaked carbon.                                           |                |
| Crinkled Carbon                                                                 | Light    | Same as for flaked carbon.                                           |                |
|                                                                                 | —        | Same as for flaked carbon, ridged, not smooth.                       | 14             |
|                                                                                 | Heavy    | Same as for flaked carbon.                                           |                |
| Smooth Carbon                                                                   | Moderate | Same as for flaked carbon.                                           |                |
|                                                                                 | Light    | Same as for flaked carbon.                                           |                |
|                                                                                 | —        | Same as for flaked carbon, smooth coating.                           | 11             |
| Sludge                                                                          | Heavy    | Same as for flaked carbon.                                           |                |
|                                                                                 | Moderate | Same as for flaked carbon.                                           |                |
|                                                                                 | Light    | Same as for flaked carbon.                                           |                |
| Varnish                                                                         | —        | Shiny, oily emulsion of carbon and oil. Can be wiped off with a rag. | 8              |
|                                                                                 | Heavy    | Approx. 1/16-inch thick.                                             |                |
|                                                                                 | Moderate | Approx. 1/32-inch thick.                                             |                |
| Clean                                                                           | Light    | Just covering.                                                       |                |
|                                                                                 | —        | Varnish or lacquer-like coating, shiny.                              | 5              |
|                                                                                 | —        | Clean — no deposit.                                                  | 0              |

## Examples 65-74

The general procedure of Examples 47-60 was repeated; however, said procedure was modified in these Examples (Examples 65-74) by including the additives shown in Tables 5 and 6 in the amounts shown for the respective Examples in said Tables 5 and 6 rather than the additives of Examples 47-60. The results obtained in Examples 65-74 are presented in Tables 5 and 6. For the purpose of comparison, the results of certain Examples (i.e., Examples 52, 56, 60, 61, 62, 63, and 64) which were reported in Table 3 or Table 4 are repeated in Table 5 or Table 6.

Corrosion Oxidation test results shown in Table 5 for Example 65 indicates that increasing the antioxidant concentration to the combined inhibitor level used in Example 60 lowered the viscosity increase. However, the higher inhibitor concentration produced an increased level of sludging, compare Example 65 with Example 48 (Table 3). Likewise, increasing the inhibitor concentration in Example 66 to the combined inhibitor level employed in Example 60 not only increased the amount of sludging, but resulted in a significantly higher viscosity increase in Corrosion-Oxidation tests, compare Example 49 (Table 3) with Example 66. A similar result was observed with the antioxidants of Examples 52 and 56 shown in Tables 3 and 5. In none of the examples shown in Table 5 was the effectiveness of a single antioxidant, regardless of concentration, equivalent to the performance obtained by the combined antioxidants of the present invention.

An examination of the overall deposit ratings obtained from Alcor High-Temperature Deposition Tests shown in Table 6 clearly shows that the improvement in cleanliness obtained as a result of alkylation (Example 62 versus Example 61) and subsequent N-substitution (Example 63 versus Example 62) of the parent secondary amine.

Results shown for Examples 61, 62 and 71 represent prior art while those for Example 63 and 72 are illustrative of the improvement in cleanliness afforded by additives of the current invention.

The improvement in oxidation stability and cleanliness obtained by the combination of antioxidants of the present invention is clearly evident by an examination of the results shown in Table 6 for Examples 74 and 64 versus that illustrated by the prior art of Example 73 which does not contain a tertiary amine. A comparison of the oxidation stability and overall deposit ratings obtained with Examples 73 and 74 clearly shows the improvement obtained by the use of the combination of an alkylated secondary amine and a tertiary amine (Example 74) selected in accordance with the teachings of the Summary or Embodiment A-1 versus that obtained by two alkylated secondary amines (Example 73). Likewise, the performance of two tertiary amines (Example 64) selected in accordance with the teaching of Embodiment A was superior to the combination of a tertiary amine and an alkylated secondary amine (Example 74).

In conclusion, as the foregoing examples show, a lubricant composition which is predominantly a carboxylic acid ester and which contains an alkylated secondary amine and an alkylated tertiary amine or, in the alternative, two alkylated tertiary amines selected as described in the Summary and Embodiments A and A<sub>1</sub> supra, exhibits improved sludging characteristics over

the prior art, and shows an acid No. change of less than 2, and a viscosity change of less than 25% in Corrosion-Oxidation Tests.

The lubricating composition of this invention as taught in the Summary and Embodiments A and A<sub>1</sub> supra also exhibit excellent oxidation stability in High-Temperature Deposition Tests as evidenced by acid number and viscosity increase while exhibiting improved cleanliness over the prior art.

10 As used herein the term "percent (%)" means part per hundred, and the term "parts" means parts by weight unless otherwise defined where used.

A mole of a substance is that quantity of the substance which contains the same number of molecules 15 of the substance as there are atoms in 12 grams of pure <sup>12</sup>C.

We claim:

1. In a lubricant composition comprising major amounts of a carboxylic acid ester lubricant, the improvement comprising the presence of,

20 a. a secondary amine having the formula;



25 35 in which R<sub>1</sub> and R<sub>2</sub> are separately alkyl groups having 4-12 carbon atoms; and

40 b. a tertiary amine having the formula;



45 50 55 or



in which  $R_4$  is an alkyl group having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen,  $A$  is  $CCl_2$ ,  $CBr_2$ ,  $Cl_2$ , or an alkylene group having about 1-7 carbon atoms, and  $R_9$  is hydrogen or an alkyl group having 4-12 carbon atoms, said secondary amine and said tertiary amine being present in an amount effective for improving oxidative stability of the ester base lubricant at temperatures up to at least 400°F.

2. The composition of claim 1 in which  $R_1$  is  $C(CH_3)_2CH_2C(CH_3)_3$ .

3. The composition of claim 1 in which  $R_2$  is  $C(CH_3)_2CH_2C(CH_3)_3$ .

4. The composition of claim 1 in which  $R_3$  is  $C(CH_3)_2CH_2C(CH_3)_3$ .

5. The composition of claim 1 in which  $R_4$  is  $C(CH_3)_2CH_2C(CH_3)_3$ .

6. The composition of claim 1 in which  $A$  is  $CH_2CH_2$ .

7. The composition of claim 1 in which  $R_9$  is  $C(CH_3)_2CH_2C(CH_3)_3$ .

8. The composition of claim 1 in which  $A$  is  $CH_2$ .

9. The composition of claim 1 in which  $R_6$ ,  $R_7$ , and  $R_8$  are hydrogen.

10. The composition of claim 1 in which said composition contains 0.5-10 parts of a phosphorus-containing ester selected from the group consisting of tricresyl phosphate, triphenyl phosphate, cresyldiphenyl phosphate, xylodiphenyl phosphate, triethyl phosphate, triethyl phosphate.

11. The composition of claim 1 in which said composition contains 0.1 part of an aminosubstituted 1,2,4-triazole.

12. The composition of claim 1 in which the carboxylic acid ester component of said composition is an ester derived from an aliphatic carboxylic acid having 3-18 carbon atoms and a polyol selected from the group consisting of trimethylolpropane, pentaerythritol, dipentaerythritol, tripentaerythritol, and neopentylglycol.

13. In a lubricant composition comprising major amounts of a carboxylic acid ester lubricant, the improvement comprising the presence of;

a. a first tertiary amine having the formula



in which  $R_4$  and  $R_5$  are separately alkyl groups having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen, and  $A$  is  $CCl_2$ ,  $CBr_2$ ,  $Cl_2$ , or an alkylene group having about 1-7 carbon atoms, and

5

10

or

30

35

40

45

50

55

60

65

b. a second tertiary amine selected from the group consisting of tertiary amines having the formula



in which  $R_4$  is an alkyl group having 4-12 carbon atoms and  $R_6$ ,  $R_7$ , and  $R_8$  are separately selected from the group consisting of  $CH_3$ ,  $C_2H_5$ , iodine, bromine, chlorine, fluorine, nitro, and hydrogen, and  $A$  is  $CCl_2$ ,  $CBr_2$ ,  $Cl_2$ , or an alkylene group having about 1-7 carbon atoms, and  $R_9$  is hydrogen or an alkyl group having 4-12 carbon atoms, said first tertiary amine and said second tertiary amine being present in an amount effective for improving oxidative stability of the ester base lubricant at temperatures up to at least 400°F.

14. The composition of claim 13 in which  $R_1$  is  $C(CH_3)_2CH_2C(CH_3)_3$ .

15. The composition of claim 13 in which  $R_2$  is  $C(CH_3)_2CH_2C(CH_3)_3$ .

16. The composition of claim 13 in which  $R_3$  is  $C(CH_3)_2CH_2C(CH_3)_3$ .

17. The composition of claim 13 in which  $R_4$  is  $C(CH_3)_2CH_2C(CH_3)_3$ .

18. The composition of claim 13 in which  $A$  is  $CH_2CH_2$ .

19. The composition of claim 13 in which  $R_9$  is  $C(CH_3)_2CH_2C(CH_3)_3$ .

20. The composition of claim 13 in which  $A$  is  $CH_2$ .

21. The composition of claim 13 in which  $R_6$ ,  $R_7$ , and  $R_8$  are hydrogen.

22. The composition of claim 13 in which said composition contains 0.5-10 parts of a phosphorus-containing ester selected from the group consisting of tricresyl phosphate, triphenyl phosphate, cresyldiphenyl phosphate, xylodiphenyl phosphate, triethyl phosphate and triisooctyl phosphate.

23. The composition of claim 13 in which said composition contains 0.1 part of an aminosubstituted 1,2,4-triazole.

24. The composition of claim 13 in which the carboxylic acid ester component of said composition is an ester derived from an aliphatic carboxylic acid having 3-18 carbon atoms and a polyol selected from the group consisting of trimethylolpropane, pentaerythritol, dipentaerythritol, tripentaerythritol and neopentylglycol.

25. The composition of claim 13 in which the first tertiary amine is selected from the group consisting of

N,N-bis-4-(1,1,3,3-tetramethylbutyl)-phenylbenzylamine  
N,N-bis-4-(1,1,3,3-tetramethylbutyl)-phenyl-2-phenylethylamine  
N,N-bis-4-(1,1,3,3-tetramethylbutyl)-phenyl-2-methylbenzylamine  
N,N-bis-4-(1,1,3,3-tetramethylbutyl)-phenyl-4-methylbenzylamine  
N,N-bis-4-(1,1,3,3-tetramethylbutyl)-phenyl-2-chlorobenzylamine  
N,N-bis-4-(1,1,3,3-tetramethylbutyl)-phenyl-4-chlorobenzylamine  
N,N-bis-4-(1,1,3,3-tetramethylbutyl)-phenyl-2,4-dichlorobenzylamine,  
N,N-bis-4-(1,1,3,3-tetramethylbutyl)-phenyl-3,4-dichlorobenzylamine,  
N,N-bis-4-(1,1,3,3-tetramethylbutyl)-phenyl- $\alpha,\alpha$ -dichlorobenzylamine,  
N,N-bis-4-(1,1,3,3-tetramethylbutyl)-phenyl-2-fluorobenzylamine,  
N,N-bis-4-(1,1,3,3-tetramethylbutyl)-phenyl-4-fluorobenzylamine,  
N,N-bis-4-(1,1,3,3-tetramethylbutyl)-phenyl-4-nitrobenzylamine, and  
N,N-bis-4-(1,1,3,3-tetramethylbutyl)-phenyl-2-phenylethylamine.

**26.** The composition of claim 13 in which the second tertiary amine is

N-4-(1,1,3,3-tetramethylbutyl)-phenyl-N- $\alpha$ -naphthylbenzylamine,  
N-4-(1,1,3,3-tetramethylbutyl)-phenyl-N- $\alpha$ -naphthyl-2-phenylethylamine,  
N-4-(1,1,3,3-tetramethylbutyl)-phenyl-N- $\alpha$ -naphthyl-2-methylbenzylamine,  
N-4-(1,1,3,3-tetramethylbutyl)-phenyl-N- $\alpha$ -naphthyl-4-methylbenzylamine,  
N-4-(1,1,3,3-tetramethylbutyl)-phenyl-N- $\alpha$ -naphthyl-2-chlorobenzylamine,  
N-4-(1,1,3,3-tetramethylbutyl)-phenyl-N- $\alpha$ -naphthyl-4-chlorobenzylamine,  
N-4-(1,1,3,3-tetramethylbutyl)-phenyl-N- $\alpha$ -naphthyl-2,4-dichlorobenzylamine,  
N-4-(1,1,3,3-tetramethylbutyl)-phenyl-N- $\alpha$ -naphthyl-3,4-dichlorobenzylamine,  
N-4-(1,1,3,3-tetramethylbutyl)-phenyl-N- $\alpha$ -naphthyl- $\alpha$ - $\alpha$ -dichlorobenzylamine,  
N-4-(1,1,3,3-tetramethylbutyl)-phenyl-N- $\alpha$ -naphthyl-2-fluorobenzylamine,  
N-4-(1,1,3,3-tetramethylbutyl)-phenyl-N- $\alpha$ -naphthyl-4-fluorobenzylamine,  
N-4-(1,1,3,3-tetramethylbutyl)-phenyl-N- $\alpha$ -naphthyl-4-nitrobenzylamine,  
N-4-(1,1,3,3-tetramethylbutyl)-phenyl-N- $\beta$ -naphthylbenzylamines,  
N-4-(1,1,3,3-tetramethylbutyl)-phenyl-N- $\beta$ -naphthyl-2-phenylethylamine,

N-4-(1,1,3,3-tetramethylbutyl)-phenyl-N- $\beta$ -naphthyl-2-methylbenzylamine,  
 N-4-(1,1,3,3-tetramethylbutyl)-phenyl-N- $\beta$ -naphthyl-4-methylbenzylamine,  
 N-4-(1,1,3,3-tetramethylbutyl)-phenyl-N- $\beta$ -naphthyl-2-chlorobenzylamine,  
 N-4-(1,1,3,3-tetramethylbutyl)-phenyl-N- $\beta$ -naphthyl-4-chlorobenzylamine,  
 N-4-(1,1,3,3-tetramethylbutyl)-phenyl-N- $\beta$ -naphthyl-2,4-dichlorobenzylamine,  
 N-4-(1,1,3,3-tetramethylbutyl)-phenyl-N- $\beta$ -naphthyl-3,4-dichlorobenzylamine,  
 N-4-(1,1,3,3-tetramethylbutyl)-phenyl-N- $\beta$ -naphthyl- $\alpha$ - $\alpha$ -dichlorobenzylamine  
 N-4-(1,1,3,3-tetramethylbutyl)-phenyl-N- $\beta$ -naphthyl-2-fulorobenzylamine,  
 N-4-(1,1,3,3-tetramethylbutyl)-phenyl-N- $\beta$ -naphthyl-4-fluorobenzylamine,  
 N-4-(1,1,3,3-tetramethylbutyl)-phenyl-N- $\beta$ -naphthyl-4-nitrobenzylamine, or  
 N-4-(1,1,3,3-tetramethylbutyl)-phenyl-N- $\beta$ -1-(1,1,3,3-tetramethylbutyl)- $\beta$ -naphthylbenzylamine.

27. A lubricant composition comprising:

- a. 100 parts of a carboxylic acid ester
  - b. 0.5-10 parts of tricresyl phosphate;
  - c. 0.5-8 parts of 4,4'-(1,1,3,3-tetramethylbutyl) di-phenylamine;
  - d. 0.5-10 parts of a tertiary amine selected from a group consisting of N,N-bis-4-(1,1,3,3-tetramethylbutyl)-phenyl-N- $\alpha$ -naphthylbenzylamine, and N,N-bis-4-(1,1,3,3-tetramethylbutyl)-phenyl-N- $\beta$ -naphthylbenzylamine; and
  - e. 0-0.5 parts of a member selected from a third group consisting of 3-amino-1,2,4-triazole, 4-amino-1,2,4-triazole, benzotriazole, 5,5-methylene-bis-(1,2,3-benzotriazole), and a lower alkyl benzotriazole.

**28. A lubricant composition comprising:**

- a. 100 parts of a carboxylic acid ester
  - b. 0.5–10 parts of tricresyl phosphate;
  - c. 0.5–8 parts of a secondary amine selected from the first group consisting of N-4-(1,1,3,3-tetramethylbutyl)phenyl- $\alpha$ -naphthylamine, and N-4-(1,1,3,3-tetramethylbutyl)phenyl- $\beta$ -naphthylamine;
  - d. 0.5–10 parts of N,N-bis-4-(1,1,3,3-tetramethylbutyl)phenylbenzylamine,
  - e. 0–0.5 parts of a member selected from a third group consisting of an amino-1,2,4-triazole, benzotriazole, 5,5-methylene-bis-(1,2,3-benzotriazole), and an alkyl benzotriazole.

29. In a lubricant composition comprising major amounts of a carboxylic acid ester lubricant, the improvement comprising the presence of;

- a secondary amine having the formula;





in which R<sub>1</sub> is an alkyl group having 4-12 carbon atoms and R<sub>3</sub> is hydrogen or an alkyl group having 4-12 carbon atoms; and

b. a tertiary amine having the formula;



in which R<sub>4</sub> and R<sub>5</sub> are separately alkyl groups having 4-12 carbon atoms and R<sub>6</sub>, R<sub>7</sub>, and R<sub>8</sub> are separately selected from the group consisting of CH<sub>3</sub>, C<sub>2</sub>H<sub>5</sub>, iodine, bromine, chlorine, fluorine, nitro, and hydrogen, A is CCl<sub>2</sub>, CBr<sub>2</sub>, Cl<sub>2</sub>, or an alkylene group having about 1-7 carbon atoms, and R<sub>9</sub> is hydrogen or an alkyl group having 4-12 carbon atoms, said secondary amine and said tertiary amine being present in an amount effective

for improving oxidative stability of the ester base lubricant at temperatures up to at least 400°F.

30. The composition of claim 29 in which R<sub>1</sub> is C(CH<sub>3</sub>)<sub>2</sub>CH<sub>2</sub>C(CH<sub>3</sub>)<sub>3</sub>.

5 31. The composition of claim 29 in which A is CH<sub>2</sub>CH<sub>2</sub>.

32. The composition of claim 29 in which R<sub>3</sub> is C(CH<sub>3</sub>)<sub>2</sub>CH<sub>2</sub>C(CH<sub>3</sub>)<sub>3</sub>.

33. The composition of claim 29 in which R<sub>4</sub> is C(CH<sub>3</sub>)<sub>2</sub>CH<sub>2</sub>C(CH<sub>3</sub>)<sub>3</sub>.

34. The composition of claim 29 in which R<sub>5</sub> is C(CH<sub>3</sub>)<sub>2</sub>CH<sub>2</sub>C(CH<sub>3</sub>)<sub>3</sub>.

35. The composition of claim 29 in which R<sub>9</sub> is C(CH<sub>3</sub>)<sub>2</sub>CH<sub>2</sub>C(CH<sub>3</sub>)<sub>3</sub>.

15 36. The composition of claim 29 in which A is CH<sub>2</sub>.

37. The composition of claim 29 in which R<sub>6</sub>, R<sub>7</sub>, and R<sub>8</sub> are hydrogen.

20 38. The composition of claim 29 in which said composition contains 0.5-10 parts of a phosphorus-containing ester selected from the group consisting of tricresyl phosphate, triphenyl phosphate, cresyldiphenyl phosphate, xylodiphenyl phosphate, triethyl phosphate, tributyl phosphate and triisooctyl phosphate.

25 39. The composition of claim 29 in which said composition contains 0.1 part of an aminosubstituted 1,2,4-triazole.

40 40. The composition of claim 29 in which the carboxylic acid ester component of said composition is an ester derived from an aliphatic carboxylic acid having 3-18 carbon atoms and a polyol selected from the group consisting of trimethylolpropane, pentaerythritol, dipentaerythritol, tripentaerythritol, and neopentylglycol.

\* \* \* \* \*